

Feb. 22, 1938.

J. O. BETTERTON ET AL

2,109,144

PROCESS OF TREATING METAL

Original Filed Aug. 17, 1933



INVENTORS  
Jesse O. Betterton  
BY Yurii E. Lebedeff  
James K. Keutk  
ATTORNEY

## UNITED STATES PATENT OFFICE

2,109,144

## PROCESS OF TREATING METAL

Jesse O. Betterton and Yuril E. Lebedeff, Metuchen, N. J., assignors to American Smelting and Refining Company, New York, N. Y., a corporation of New Jersey

Application August 17, 1933, Serial No. 685,586  
Renewed August 28, 1937

5 Claims. (Cl. 75—78)

This invention relates to an improved process of treating metals to effect the removal therefrom of contaminating metal values.

The invention provides a process for treating 5 molten metal at low temperatures by which contaminating metals are readily and effectively removed without the formation of excessively large amounts of complex slags or drosses.

Among other features, the invention contemplates the establishment and maintenance of a liquid two phase equilibrium system comprising the molten metal undergoing treatment and a slag which is fluid at the operating temperatures employed and also non-reactive with respect both 15 to the metal treated and reagents, if any, used.

It is, of course, well known that as a general rule the degree of solubility of one metal in another varies with the temperature and that fact is commonly taken into consideration in practising ordinary liquidation separations. Again, 20 it is common practise to remove impurities from metals by incorporating suitable reagents therein which will selectively react with the impurities and permit their accumulation and removal as drosses. However, these processes or combinations thereof as generally practised usually have some inherent disadvantages among which may be mentioned the formation of large or excessive 25 quantities of dross, the difficulties encountered in treating the dross arising from both the large quantity thereof and its physical and chemical composition, the excessive oxidation of the metal and the loss of efficiency due either to the chemical conversion of relatively large amounts of the 30 metal treated to undesired compounds or its mechanical entrapment in the impurity being removed.

The foregoing and other disadvantages are overcome and new and useful results obtained 40 by employing a two phase equilibrium system in accordance with the present invention. In general, the improved process may be practised by covering a molten bath of the metal to be refined with a suitable slag, that is, one which is chemically inert with reference both to the metal being refined and the contaminants being removed 45 therefrom and which is and remains fluid at the operating temperature employed. By agitating the bath, equilibrium is established and maintained between the different phases of the system. In case the equilibrium value for a particular separation is not sufficiently low, suitable reagents may be employed to lower such value as will be hereinafter described.

55 The drawing accompanying the specification

is a flow sheet illustrating the process of the invention.

In order to more fully illustrate the many novel features and advantages of the invention several specific examples of the process as applied to 5 decopperizing lead are given, although it is to be understood that the invention is not limited thereby as it may be utilized in conducting other refining operations, such as, for example, the de-silverization of lead.

10

*Example 1*

In this instance impure blast furnace lead was melted down in a cast iron kettle, the dross skimmed and the bath sampled. The total weight 15 of the bath was 188.5 lbs. and was shown by analysis to contain 0.90% copper, 0.31% arsenic, 1.83% antimony, and 392 oz./ton doré. At a temperature of 850° F., a slag comprising 0.44 lb. of zinc chloride and 0.15 lb. of sodium chloride 20 was added to the surface of the bath and allowed to melt. The bath was then agitated by an ordinary mixing machine beginning at a temperature of 725° F. and continued until the temperature had fallen to 660° F. At this stage a preheated 25 hand operated press was placed in the kettle and the metallic mushy liquate intermixed with the chloride slag was skimmed into the press. The bath was pressed clean at 595° F. and the pressed dross weighing only 6.25 lbs. was found to analyze 30 25.3% copper. An analysis of the final bath which weighed 182.2 lbs. showed 0.06% copper, 0.08% arsenic, 1.61% antimony and 392.0 oz./ton of doré.

35

*Example 2*

It will be noted that in Example 1 the copper content was reduced to 0.06%, which figure represents the approximate equilibrium value for that system. In order, then, to lower that value 40 and further decrease the copper content in accordance with the invention, the 182.2 lbs. of lead were treated as follows: the bath was reheated to 660° F. and 0.22 lb. of zinc chloride and 0.08 lb. of sodium chloride added and allowed to melt at 640° F. At this stage, 0.360 lb. of zinc 45 dust were incorporated in the bath, after which the mushy dross was pressed as in Example 1. The pressed dross weighed 0.9 lb. and analyzed 6.7% copper while the bath weighed 181.7 lbs. and contained 0.03% copper, 0.08% arsenic, 50 1.67% antimony and 386.5 oz./ton of doré.

45

50

55

*Example 3*

In this instance, a bath of copper-bearing lead weighing 153.7 lbs. after melting down and skim-

ming and analyzing 0.069% copper was mixed with a molten slag comprising 0.1 lb.  $ZnCl_2$  and 0.02 lb.  $NaCl$  at 650° F. Thereafter, 0.32 lb. of powdered zinc were incorporated in the bath and the temperature lowered to the freezing point. The molten metal was then tapped from the kettle and found to contain only 0.012% copper.

*Example 4*

10 One hundred, forty-four and eighth-tenths lbs. of lead were melted in a small cast iron kettle and 1.1 lbs. of dross formed during the melting down operation were skimmed at a temperature of 660° F. By analysis, the bath was found to 15 contain 0.115% copper. Powdered sulfur to the amount of 0.175 lb. was added to the bath at a temperature of 630° F. and thoroughly incorporated therein. This operation was performed in 20 22 minutes, at which time the dross weighing 17.5 lbs. or 12.08% by weight of the original lead treated was removed from the bath at a temperature of 660° F. The molten lead bath was then sampled and found to contain 0.06% copper. At this stage, a slag comprising 1.3 lbs. of 25 zinc chloride and 0.3 lb. of sodium chloride was added to the surface of the bath and allowed to completely melt at 650° F. The 17.5 lbs. of mushy dross were returned to the bath, the contents of the kettle mixed by hand for a few minutes and 30 the slag skimmed from the bath. The gross weight of the slag was only 3.5 lbs. or a net weight of 1.9 lbs., equivalent to 1.31% by weight of the lead originally treated. The bath analyzed 0.06% copper.

*Example 5*

One hundred fifty-eight and one-half lbs. of copper-bearing lead were melted in a kettle and the dross formed during the melting operation (1.1 lbs.) removed. By analysis the bath contained 0.12% copper. After adding a slag comprising 0.66 lb. of zinc chloride and 0.25 lb. of sodium chloride, sulfur to the amount of 0.66 lb. was incorporated in the bath at a temperature of 45 630° F. The slag, weighing 2.3 lbs., was skimmed from the surface of the bath and a sample of the bath taken which analyzed 0.069% copper. At this stage, a second slag comprising 0.1 lb. of zinc chloride and 0.2 lb. of sodium chloride was added to the surface of the bath. Thereafter, 0.32 lb. of powdered zinc was incorporated 50 in the molten lead and the temperature lowered to a point approaching the freezing point of lead. The molten metal was then tapped from the kettle and found to contain only 0.012% copper and 55 0.06% zinc.

From the several preceding specific examples it will readily be appreciated that new and improved results are obtained when metals are 60 treated in accordance with the two liquid phase process of the present invention. The ease with which contaminants in metal may be reduced to their solubility limits at the temperature employed without the production of large amounts 65 of dross or recourse to any reagents is clearly exemplified by Example 1. Examples 2 and 3, among other features, illustrate how the amount of a contaminant may readily be reduced simply by employing a reagent which will lower the 70 equilibrium value. The marked reduction in dross produced by employing the equilibrium system in combination with a reagent is amply brought out in Example 4, while Example 5 illustrates the consecutive use of reagents which im-

part different equilibrium values to a given two phase liquid system.

It is believed that the improved results obtained by the invention may be in a large part explained on the theory that providing a suitable fluid slag on the molten metal optimum conditions of equilibrium between the bath and slag with relation to the solubility of the contaminant being removed are at all times maintained. Instead of forming a solid dross upon the surface of the 10 bath, the contaminant is maintained in a liquid state and the metal which ordinarily is enmeshed in the dross is allowed to reenter the bath while at the same time the contaminant being in amounts in excess of the solubility of same 15 in the bath at the temperature employed remains in the liquid slag. Hence, it follows that while a mixture of zinc chloride and sodium chloride has been specifically mentioned by way of illustration, any slag, which is fluid at the temperatures employed and which will not react with the metal or reagents, if any, used, may be utilized. It is, of course, obvious that the slag will also serve the secondary purpose of preventing oxidation of the bath and reagents.

It is obvious that in addition to decreasing the amount of dross formed, the invention facilitates the handling and processing of the slag containing the contaminants removed from the metal both from the standpoints of quantity and physical composition. For example, slags obtained by decopperizing lead may be leached with water to remove the soluble constituents therefrom and the residue smelted to produce a concentrated copper matte which is readily processed for the 35 recovery of copper.

While certain novel features of the invention have been disclosed and are pointed out in the annexed claims, it will be understood that various omissions, substitutions and changes may be 40 made by those skilled in the art without departing from the spirit of the invention.

What is claimed is:

1. In the process of removing copper from lead by incorporating a decopperizing reagent in 45 the molten lead whereby copper is concentrated as a dross, the improvement which comprises conducting the operation in the presence of a fluid slag comprising a mixture of zinc chloride and sodium chloride thereby concentrating the 50 copper in a combined slag and dross of small weight.

2. A process of refining copper-containing lead, which comprises forming a molten bath of the lead, producing on the said bath a molten slag 55 layer comprising zinc chloride and sodium chloride, the slag layer remaining fluid at the temperature of operation and being substantially inert with respect to the lead in the bath, producing a dross of the copper contained in the lead, 60 and contacting the bath and slag to concentrate the dross in the slag, thereby establishing conditions of equilibrium between the bath and slag, the said slag being adapted to retain the dross while returning to the bath the lead which was en- 65 trapped in the dross.

3. A process of refining copper-containing lead, which comprises forming a molten bath of the lead, producing on the said bath a molten slag 70 layer comprising zinc chloride and sodium chloride, the slag layer remaining fluid at liquation temperature of the bath and being substantially inert with respect to the lead in the bath, liquating the bath to produce a dross of the copper contained in the lead, and agitating the bath and 75

5 slag to concentrate the dross in the slag, thereby establishing conditions of equilibrium between the bath and slag, the said slag being adapted to retain the dross while returning to the bath the lead which was entrapped in the dross.

10 4. A process of refining copper-containing lead, which comprises forming a molten bath of the lead, producing on the said bath a molten slag layer comprising zinc chloride and sodium chloride, the slag layer remaining fluid at the temperature of operation and being substantially inert with respect to the lead in the bath, adding to the bath a reagent for the copper adapted to produce a separation of the copper from the bath 15 as a dross, and agitating the bath and slag to concentrate the dross in the slag, thereby establishing conditions of equilibrium between the bath and slag, the said slag being adapted to retain

the dross while returning to the bath the lead which was entrapped in the dross.

5 5. The process for refining lead by liquation with production of a minimum amount of dross which comprises forming a molten bath of the 5 lead to be liquated, establishing on the bath a fluid, salt slag which is chemically non-reactive with respect to lead and which will retain its fluidity throughout the liquating temperature range, bringing the bath and slag into equilibrium 10 with respect to the impurities to be removed by mixing the bath and slag while simultaneously cooling same thereby concentrating impurities in the slag with minimum production of dross and effecting a separation between the refined lead 15 and the slag.

JESSE O. BETTERTON.  
YURII E. LEBEDEFF.